

## UNITED STATES PATENT OFFICE.

ROBERTSON P. DRUMMOND, OF LOS ANGELES, CALIFORNIA, ASSIGNOR TO PACIFIC CAST IRON PIPE & FOUNDRY COMPANY, OF LOS ANGELES, CALIFORNIA, A CORPORATION OF CALIFORNIA.

## COMPOSITION OF MATTER.

No Drawing.

Application filed August 7, 1925. Serial No. 48,880.

This invention relates to a process and method of forming and producing special alloy metal. In particular the invention relates to an alloy metal which is more abrasive in nature than shock-resisting. The invention has for an object the provision of a metal which will prove superior to present known metals where great abrasive action is necessary, such as in all grinding and crushing work, and more particularly as mill liners, crusher jaws, disc grinders, roll grinders, cement mills and gyratory crushers.

Another object is the provision of a metal which has remarkable wearing qualities without being brittle.

Another object is the provision of a metal which will not pean.

A further object is the provision of a metal which will give 25% more wear than manganese steel in all castings for abrasive purposes.

A further object is the provision of a metal alloy which is magnetic.

The metal can readily be made largely from waste metals such as old tin cans, automobile fenders, galvanized cuttings and clippings and steel turnings, as well as out of scrap steel in any form. The metal is melted as in ordinary steel practice and the necessary alloy elements added. The analysis of the metal is as follows:

|            | Per cent.  |
|------------|------------|
| Carbon     | 1.75 to 2  |
| Manganese  | 6.25 to 8  |
| Silicon    | 1.50 to 2  |
| Phosphorus | .03 to .06 |
| Sulphur    | .01 to .03 |

The remaining percentage to make 100 per cent is of course made up by the use of iron. At first sight it may appear that a metal containing the combination of ingredients above set forth would be worthless, but the whole combination gives a structure containing cementite, martinsite, pearlite and some graphite. Photomicrographs have shown that the pearlite and martinsite in this metal

are combined, which is a most unusual feature. Ordinarily martinsite is produced by a rapid quenching of high carbon steel from a slightly higher temperature than the maximum temperature of the critical interval. Martinsite is also found in the carbonized regions of case-hardened soft steels, hardened by quenching. With the present metal, however, the metal is not hardened by quenching and still martinsite is produced. Therefore this is a distinctive metal, because so far as the inventor is aware no other metal will show pearlite and martinsite together with the production of the martinsite without the usual quenching. In one particular the metal of the invention is what may be termed a contradictory metal because from a metallurgical standpoint a manganese content of between 6.25% to 8% is the weakest point of manganese in steel. A silicon content of 1.50% to 2% is also a dangerous point in true steel, while a carbon content at 2% is dangerous. The whole combination, however, gives a metal which is very valuable for the purpose intended.

I have found that the metal can be conveniently made within the limits of the percentages given for the various alloy elements in the analysis.

Having thus disclosed my invention, I claim and desire to secure by Letters Patent:

1. A new composition of matter, comprising in combination: iron, carbon 1.75 to 2%, manganese 6.25 to 8%, and silicon 1.50 to 2%.

2. A new composition of matter, comprising, in combination: iron, carbon 1.75 to 2%, manganese 6.25 to 8%, silicon 1.50 to 2%, and phosphorus .03 to .06%.

3. A new composition of matter, comprising, in combination: iron carbon 1.75 to 2%, manganese 6.25 to 8%, silicon 1.50 to 2%, phosphorus .03 to .06%, and sulphur .01 to .03%.

In testimony whereof, I have signed my name to this specification.

ROBERTSON P. DRUMMOND.